

## UNITED STATES PATENT OFFICE

2,101,647

## FLOTATION PROCESS

Herbert P. A. Groll, Oakland, Calif., assignor to  
Shell Development Company, San Francisco,  
Calif., a corporation of Delaware

No Drawing. Application August 28, 1933,  
Serial No. 687,196

8 Claims. (Cl. 209—166)

In my copending application, Serial No. 654,253, filed January 30, 1933, of which this case is a continuation-in-part, I have described the production of novel compounds, i. e. unsaturated 5 xanthates of alcohols containing at least four carbon atoms to the molecule. Amongst others, I have described isobut enyl xanthate, pentenyl and hexenyl xanthates and the like.

I have discovered that these compounds, 10 whether of straight chain or forked chain character, are useful in flotation processes as promoters, particularly in froth flotation operations.

The alkali-metal salts of these unsaturated xanthic acids, particularly the sodium and potassium salts are most preferred.

The promoters may be utilized with any of the well-known accessory reagents such as depressors, regulators, frothers and activators. The unsaturated xanthates permit operation in an 20 alkaline medium and are preferably added in the form of a solution. The unsaturated xanthates may be used alone or with other promoters, including the use of two or more unsaturated xanthates.

25 *Example 1*

A free milling gold ore of a value of \$33.60 per ton, 90% of the gold being present in the free state, was ground to less than 65 mesh. The 30 pulverized ore was subjected to a standard flotation operation using 0.1 lb. isobut enyl xanthate and 0.005 lb. pine oil per ton for a period of nine minutes. 4.17% of concentrate were recovered having a value of \$469.60 per ton. The tailings 35 contained gold to the value of \$8.00 per ton.

25 *Example 2*

The same ore as used in Example 1 was treated under the same conditions, but using a mixture 40 of primary and secondary iso-octenyl xanthate. The concentrate in this case amounted to 4.70% having a value of \$412.00 per ton, the tailings having a value of \$9.60 per ton.

Besides the unsaturated xanthates, previously 45 mentioned, I may use primary and/or secondary unsaturated xanthates such as allyl xanthate, crotyl xanthate, primary isopentenyl xanthate, isopropenyl methyl carbinyl xanthate, cyclohexenyl xanthate, phenyl, isopropenyl carbinyl 50 xanthate, etc. as flotation promoters, the particular promoter being more or less dependent on the character of the ore undergoing treatment, the mineral content thereof, the hydrogen-ion concentration of the liquid, the tendency of 55 the gangue materials to be carried along with the

froth, etc. Those containing at least four carbon atoms to the molecule are particularly suitable for certain ores and those containing an unsaturated tertiary carbon atom directly linked to the carbinol group are especially 5 desirable.

Copper, zinc, lead and similar ores also may be treated with my novel promoters.

I claim as my invention:

1. A method of recovering minerals from ores 10 which comprises subjecting an ore to a froth flotation operation in the presence of an iso-alkenyl xanthate.

2. A method of recovering minerals from ores 15 which comprises subjecting an ore to a froth flotation operation in the presence of an unsaturated aliphatic xanthate containing not more than five carbon atoms in the aliphatic radical.

3. A method of recovering minerals from ores 20 which comprises subjecting an ore to a froth flotation operation in the presence of an unsaturated aliphatic xanthate containing four carbon atoms to the molecule.

4. A method of recovering minerals from ores 25 which comprises subjecting an ore to a froth flotation operation in the presence of isobut enyl xanthate.

5. A method of recovering minerals from ores 30 which comprises subjecting an ore to a froth flotation operation in the presence of a xanthate of an unsaturated alcohol containing an unsaturated tertiary carbon atom linked directly to the carbinol group.

6. A method of recovering minerals from ores 35 which comprises subjecting an ore to a froth flotation operation in the presence of an iso-pentenyl xanthate.

7. A method of recovering minerals from ores 40 which comprises subjecting an ore to a froth flotation operation in the presence of an allyl xanthate.

8. A method of recovering minerals from ores 45 which comprises subjecting an ore to a froth flotation operation in the presence of an unsaturated xanthate of the general formula.



wherein R represents an isoalkenyl radical, an alkenyl radical at least one hydrogen atom of which is substituted by a cyclic organic radical, or a straight chain alkenyl radical containing less than six carbon atoms, and M represents a 50 metal.

HERBERT P. A. GROLL. 55